

July 4, 1944.

H. S. GOODWIN

2,353,027

BITUMINOUS ROAD PAVEMENTS

Filed May 3, 1940

Cross Sectional View of Road Construction  
Employing Treated Cotton Fabric

- a - Surface or Wearing Course
- b - Asphalt Treated Graded Aggregate Base
- c - Treated Fabric
- d - Primed Sub-grade



Henry S. Goodwin Inventor

By P. D. Young Attorney

## UNITED STATES PATENT OFFICE

2,353,027

## BITUMINOUS ROAD PAVEMENT

Henry S. Goodwin, East Bound Brook, N. J., assignor to Standard Oil Development Company, a corporation of Delaware

Application May 3, 1940, Serial No. 333,156

10 Claims. (Cl. 94—9)

This invention relates to improvements in bituminous road pavements and particularly in the method of laying bituminous road pavements.

In laying bituminous road pavements, the use of cotton fabric is gradually increasing, especially in pavements that are subjected to very heavy traffic where the cotton acts as a binding and shock-absorbing agent. These pavements also are adapted to be used as linings in canals, both for the bottoms of the canals and also the sides. A disadvantage found in the use of cotton fabric and, in fact, in the use of other fibrous material is that the fabric absorbs some of the moisture from the base with the result that the adhesivity of the fabric and the bituminous material is materially reduced. The bituminous material tends to part from the fabric and also the fabric tends to stretch and/or weaken due to rotting. Attempts have been made to overcome these difficulties by waterproofing this fabric by saturating with a bituminous composition such as a good grade of soft blown asphalt with or without first pre-treating with a bituminous saturating compound. Even then the treated fabric and the top surface bituminous composition does at times tend to part.

An object of this invention is to overcome the above-mentioned difficulties currently encountered from the use of cotton cloth in pavements by the use of a fabric which has been made water repellent by impregnation with aluminum stearate.

Another object of this invention is to provide a pavement which possesses a greater adhesion of the ingredients in the pavement with a certain measure of vibration-absorbing property.

Still another object of this invention is to provide a pavement in which the bond between a fibrous fabric used in the pavement and the bituminous composition is greatly improved.

A further object of this invention is to provide a pavement that will withstand weathering, such as rain, frost and snow, over prolonged periods of time.

According to this invention, cotton fabric or other fibrous material that is to be used in the construction of pavements, may be prepared in any manner which will leave the fibers of the material sufficiently impregnated with aluminum stearate to render them substantially waterproof. One known method by which this is accomplished is to first saturate the cloth or fibrous material with an aqueous solution of aluminum acetate of about 4 to 5 Baumé gravity, then to pass the saturated material into a bath containing an

aqueous solution of a water-soluble stearate soap, such as sodium stearate, to precipitate aluminum stearate in the fibers of the fabric, and to then free the fabric from the excess soap solution by rinsing or washing. The fabric is then subsequently dried by means of heat and/or pressure in a suitable manner. A 2% alum solution or similar type water-soluble aluminum salt solution is at times used as a fixing agent, through which the fabric is passed just after the precipitation of the aluminum stearate, and prior to the final washing or rinsing step.

The aluminum stearate impregnated fabric is then laid on the surface of a road or canal base that has previously been prepared. If desired, the base may be primed with a flux oil or cutback liquid asphalt preparation and allowed to cure for about a day before the addition of the fibrous fabric. Fine, medium, or coarse mesh fabrics may be used.

The fabric may be treated with an asphalt cutback oil, and sand spread on top. Another method is to cover fibrous fabric material with a good coating of asphalt and cut stone which is then rolled and finally given a top coat of asphalt.

When used in lining canals, the base is generally given a prime coat of road oil and a coating of a fluid asphalt. The coated fabric is then laid and covered with asphalt upon which a seal-coat of asphalt together with a mineral, such as stone chips, is added.

Hot asphalt applications may be used in coating the fibrous fabric after it is laid or, if desired, a composition of flux oil and powdered asphalt with or without mineral aggregate may be used as a surface coating on the fibrous fabric which, on being rolled, amalgamate to form a stronger paving. Wetting agents, such as lead naphthenate, lead sulfonate, or free fatty acids, may likewise be incorporated in the flux or asphaltic material that is used.

These bituminous road pavements are especially useful wherever extensive areas are required to be paved and maintained smooth, such as airplane port fields, kennel floors and runs, driveways, garage floors, tennis courts, etc.

I claim:

1. A pavement comprising as a supporting substructure a fibrous material which has been previously impregnated with a metallic stearate and a top wearing surface of bituminous material.

2. A pavement comprising a bituminous oil treated substructure, a fibrous material which has been previously impregnated with aluminum

stearate, and a top layer of asphalt and mineral aggregate.

3. The method of laying a pavement which comprises leveling a substructure, laying on the substructure a fibrous material which has been previously impregnated with aluminum stearate and covering the fibrous, impregnated material with an asphalt composition.

4. A method of laying a pavement which comprises preparing a substructure, treating it with an asphaltic mineral oil, laying on the asphaltic-treated substructure the asphalt coated fabric previously impregnated with aluminum stearate, and covering the coated fabric with a mixture of mineral aggregate and bituminous material.

5. A method of laying a pavement according to claim 4 in which the bituminous material used in bonding the mineral aggregate contains a wetting agent.

6. A method of laying a pavement which comprises coating a substructure with an asphaltic flux oil, laying on the substructure a cotton fabric that had been impregnated with aluminum stearate and covering the cotton fabric with a mixture of mineral aggregate, powdered asphalt and flux oil, and compacting the mixture cold by the application of pressure.

7. A method of laying a pavement according to claim 6 in which the cotton fabric is impregnated with aluminum stearate by saturating the cotton fabric with a water solution of an alumi-

num salt and then passing the aluminum salt treated fabric through a bath containing an aqueous solution of sodium stearate, after which the fabric is dried.

8. A method of laying a pavement which comprises saturating a fibrous material with a water solution of an aluminum salt and then passing the aluminum salt treated fabric through a bath containing an aqueous solution of sodium stearate, pressing to remove most of the liquids, drying the fabric, coating a substructure with an asphalt flux oil, laying on the asphaltic flux oil treated substructure the aluminum salt treated dry fabric, coating the aluminum salt treated dry fabric with a mixture of mineral aggregate, powdered asphalt and flux oil, and compacting the mixture by the application of pressure.

9. A method of laying a pavement according to claim 8 in which the fibrous material is a cotton fabric.

10. A method of laying a pavement which comprises treating a fibrous material with a water solution of a water-soluble aluminum salt and then passing the aluminum salt treated fabric through a bath containing an aqueous solution of sodium stearate, drying the fabric, coating a substructure with an asphaltic flux oil, laying on the asphaltic flux oil treated substructure the dry fabric and covering the dry fabric with a hot mixture of mineral aggregate and asphalt.

HENRY S. GOODWIN.